

## UNITED STATES PATENT OFFICE

ALAN S. HAWKESWORTH, OF WASHINGTON, DISTRICT OF COLUMBIA

## MANUFACTURE OF NITROCELLULOSE SMOKELESS POWDER

No Drawing.

Application filed June 13, 1930. Serial No. 461,056.

This invention has for its object, the modification, to suit present working conditions and routine, of the process of such manufacture set forth in my prior Patent 1,713,505; 5 granted to me 14th May, 1929.

After the nitration of the cotton fibre, or cellulose, it must be thoroughly washed in water to eliminate the exceedingly dangerous free nitric acid and then must be dried 10 or dehydrated. In my previous Patent 1,713,505 I accomplished this by employing an excess of my combined "dryer, solvent, and stabilizer," mono-nitro-toluene, which excess had then to be eliminated, by centrifuging 15 or some similar method. But in this improved process I am only going to employ the irreducible minimum of around 6% mono-nitro-toluene so that the washed and damp nitrocellulose is now dehydrated by the addition of alcohol in the present customary way.

And when the nitrocellulose is so dried, and ready for the solvent, I now use only the stated irreducible minimum, of around 6% or 25 so by volume, of mono-nitrotoluene; and add say three or four times as much ether to make the compound "excess solvent". To every 100 parts by volume of the nitrocellulose, there are added about 6 or 7 parts by volume of 30 mono-nitro-toluene and say 20 parts by volume of ether; or whatever excess may be needed to make a smooth, easily workable colloid or paste, which excess of solvent also ensures the complete dis-solution or solution 35 of the nitrocellulose.

Having so dissolved thoroughly the nitrocellulose and made my desired powder grain pattern—American, strip, or any other—from the soft paste; the completed powder 40 grain is then baked at a very moderate temperature (around "blood heat") in the drying oven, and all the superfluous ether solvent evaporated out. Since the mono-nitro-toluene boils at the high temperature of 220.4° 45 Cent. or 428.7° Fahr. it is absolutely unaffected by the moderate temperature that drives out and evaporates the ether. The non-evaporable mono-nitro-toluene is thus left hermetically sealing each and every molecule of the nitrocellulose in its own water- 50

proof and cushioned cell, making an absolutely safe powder that cannot deteriorate from elapsed time, or extreme climatic conditions, and, incidentally, also being incapable of exploding spontaneously, through static 55 electric sparks self generated by friction. These valuable advantages, as stated in my previous Patent 1,713,505, are due to the employment of the mono-nitro-toluene as my solvent, chemically and intimately coating, 60 as a solvent, each individual molecule of the nitrocellulose; and thus fulfilling efficiently, the office of a stabilizer, and not merely using it, like other greasy "stabilizers", as an after 65 addition and mechanical admixture, after the powder is made whereby no such intimate coating is possible.

But when the mono-nitro-toluene alone is used, the necessary excess (ensuring complete solution of the nitrocellulose) is difficult to 70 remove, and by this present use of a compound solvent, composed of the minimum needed mono-nitro-toluene and the excess solvent of ether, or other easily evaporable solvent, my obtain a paste that, when the desired powder 75 grain is moulded, can be easily and quickly dried and hardened in the drying oven, and drying and hardening, however, absolutely ceases, when all the ether is driven off, and the non-evaporable mono-nitro-toluene left be- 80 hind to do its preserving work, a state that will continue unaltered, instead of the drying out and hardening still continuing while in storage, to the danger point as with the present smokeless powder; where the ether solvent 85 is employed alone in which some greasy "stabilizer" is added after the powder is made.

I claim:

The process of making nitrocellulose smokeless powder which comprises, the addition as a solvent and stabilizer of mono-nitro-toluene of around at least 6% by volume of the finished powder grain as the irreducible minimum, needed to completely coat each molecule of the nitrocellulose, together with the addition of an easily evaporable solvent sufficient to make a compound solvent that will completely dissolve the nitrocellulose 90 into a smooth paste, and evenly distribute 95 100

the mono-nitro-toluene, then moulding the said paste into the desired powder grain, and driving off the excess evaporable solvent from the finished powder grain by means of 5 moderate heat, thereby leaving the non-evaporable mono-nitro-toluene coating over each and every one of the nitrocellulose molecules.

ALAN S. HAWKESWORTH.

10

15

20

25

30

35

40

45

50

55

60

65